

G. MICHAUD & E. DELASSON,  
MANUFACTURE OF FILAMENTS FOR ILLUMINATING AND HEATING PURPOSES,  
APPLICATION FILED MAY 6, 1908.

972,893.

Patented Oct. 18, 1910.



Witnesses:-

C. H. Crawford  
E. Schallinger

Inventors:-

Georges Michaud  
Eugène Delasson  
By B. J. Siple Attorney

# UNITED STATES PATENT OFFICE.

GEORGES MICHAUD AND EUGÈNE DELASSON, OF MONTREUIL, SEINE, FRANCE.

## MANUFACTURE OF FILAMENTS FOR ILLUMINATING AND HEATING PURPOSES.

972,893.

Specification of Letters Patent. Patented Oct. 18, 1910.

Application filed May 6, 1908. Serial No. 431,204.

*To all whom it may concern:*

Be it known that we, GEORGES MICHAUD and EUGÈNE DELASSON, citizens of the Republic of France, and residents of Mon-treuil-sous-Bois, Seine, France, have invented certain new and useful Improvements in the Manufacture of Filaments for Illuminating and Heating Purposes, of which the following is a specification.

10 We have disclosed in the specification forming a part of our application for Letters Patent, Serial No. 399,963, filed October 30, 1907, the composition of and the process for manufacturing refractory filaments to be used for incandescent gas lighting.

15 The invention forming the subject matter of the present application for Letters Patent, relates to certain modifications in the proportions of the primary material constituting the said filaments; and it also embodies improvements in the method of treating the filaments.

20 A typical ratio for the quantities used of the radiant substances which produces good results, is as follows:

|                           |      |
|---------------------------|------|
| Oxid of thorium           | 93   |
| Oxid of cerium            | 1 95 |
| Oxid of glucinum          | 1    |
| Oxid of aluminium         | 4    |
| Silicate of aluminium     | 1 5  |
| Oxid of chromium (traces) |      |

25 This example of the composition of the filament is given for the purpose of showing how the proportions may vary while the materials selected remain the same.

30 It should be understood that each of these oxids may be replaced by any one of the oxids of the same series, or by a mixture of several oxids of the same series. Thus, the oxid of aluminium might be replaced by the oxids of silicon, of magnesium, or of calcium, either separately or mixed together, and 35 under the same conditions, the oxids of thorium and of glucinum might be replaced by the oxids of cerium, of zirconium, of erbium or others of the series, either separately or mixed together.

40 As is indicated in the specification forming part of our prior application for Letters Patent herein before referred to, the materials are agglutinated into a pasty mass, converted into filaments by means of draw plates or nozzles and subjected to a baking 45 action. This latter operation, however, in

accordance with the present invention, comprises two periods, which entails a modification of the means originally devised.

The accompanying drawing shows partly 60 in elevation and partly in section the novel device adapted for the fusion of the filaments.

Referring particularly to the drawing, E represents a nozzle into which the agglutinated material is placed, and from the lower end of which it is pressed in the form of a filament D. Below the nozzle E is the chamber F in which two or more oxyhydrogen blow-pipes G converge, the pipes H and O 70 connecting with sources of hydrogen and oxygen supply, respectively. The filament D on leaving the nozzle E is therefore subjected to the action of these convergent oxyhydrogen flames and is there fused for the 75 first time (or the fusion is initiated) then, continuing its movement, it enters an electric furnace, A, and is protected by the infusible tube C of carborundum and when in proximity to the electric arc, it attains a 80 pasty condition of fusion which insures the perfect refining of the material. This novel arrangement, which is herein disclosed, in connection with a vertical furnace, is also 85 obviously applicable to furnaces of other types, the oxyhydrogen blow-pipes being placed between the outlet of the nozzles and the electric arc.

In the prior application referred to, we have described black soap as the agglutinant, 90 and in addition thereto, it may now be stated, that among the substances which will fulfil the same purpose, an agglutinant composed of 9 parts of arabin, and 1 part of ammonia soap can successfully be employed. 95

We claim:

1. The process of manufacturing incandescent filaments, which consists in agglomerating material, forming the same into a filament, subjecting said filament to the action of a gaseous flame whereby an initial fusion is produced, and afterward subjecting said filament to the heat from an electric arc. 100

2. The process of manufacturing incandescent filaments, which consists in agglomerating material, forming the same into a filament, subjecting said filament to an oxyhydrogen flame, and afterward subjecting said filament to the heat from an electric arc. 105

3. A filament comprising oxid of thorium, 110 oxid of cerium, oxid of glucinum, oxid of

chromium, oxid of aluminium, and silicate of aluminium.

4. A filament comprising a plurality of radiant materials, and an agglutinant composed of arabin and ammonia soap.

5. A filament comprising a plurality of radiant materials, and an agglutinant composed of substantially nine parts of arabin and one part of ammonia soap.

10. 6. A filament comprising substantially ninety-three parts oxid of thorium, one part

oxid of cerium, one part oxid of glucinum, four parts oxid of aluminium, and one part silicate of aluminium.

In testimony whereof we affix our signatures in presence of two witnesses.

GEORGES MICHAUD.  
EUGÈNE DELASSON.

Witnesses:

MILTON BRAIN,  
VICTOR MONTRAY.